

R. A. HADFIELD.

ARMOR PLATE.

APPLICATION FILED MAR. 31, 1909. RENEWED AUG. 6, 1913.

1,089,638.

Patented Mar. 10, 1914.

Fig. 1.



Fig. 2. Fig. 3.



Fig. 4.



Witnesses:

J. M. Millward  
H. L. Brislain

Inventor

Robert Abbott Hadfield,  
By his Attorney  
Alfred Wilkinson.

# UNITED STATES PATENT OFFICE.

ROBERT ABBOTT HADFIELD, OF SHEFFIELD, ENGLAND.

## ARMOR-PLATE.

1,089,638

Specification of Letters Patent. Patented Mar. 10, 1914.

Application filed March 31, 1909, Serial No. 487,041. Renewed August 6, 1913. Serial No. 783,412.

To all whom it may concern:

Be it known that I, ROBERT ABBOTT HADFIELD, a subject of the King of Great Britain, residing at Parkhead House, Sheffield, 5 in the county of York, England, have invented new and useful Improvements in Armor-Plate, of which the following is a specification.

In battleships and like armor clad ships, 10 the armor is at present built up of a number of rolled or forged steel plates each of which is usually of uniform section throughout its depth. The manufacture of such plates involves long, difficult and costly operations and where such plates have to be 15 made of curved shape or of taper section for part of their depth, as is sometimes required, this adds considerably to the difficulties and cost. Furthermore, such armor 20 plates can only be produced practically of such dimensions that at least two of them placed vertically edgewise one on the other are necessary to obtain the full depth of armor required, so that great care and much 25 labor is required in securely holding the plates in position and the resulting armor contains in addition to vertical joints many horizontal ones which result in additional lines of weakness in the armor.

Now the present invention has for object 30 to provide a battle ship or like armor clad vessel (hereinafter referred to as a battleship) with armor that shall offer very great resistance to penetration and fracture, which 35 can be constructed and applied in a quicker, cheaper and more effective manner than the rolled or forged armor heretofore employed, and the several sections of which can be readily made of any desired section to allow 40 of the material being disposed to the best advantage to resist attack with the minimum of weight, and of any desired curvature to suit the different parts of the battleship to which they are to be applied, and 45

which can be made of such superficial dimensions as to avoid the presence in the armor built up of such plates of any horizontal lines of division or joints. To this end, according thereto, a battleship is 50 constructed with armor built up of plates or sections of steel or steel alloy, such as nickel steel and nickel chromium steel that is capable of being cast to the desired shape and of offering great resistance to perforation 55 and fracture. The plates or sections are preferably made of nickel-chromium steel

alloy of the kind known as "Era steel," as made by Hadfield's Steel Foundry Company Limited, of Sheffield, such steel having substantially the composition set forth in the 60 specification of British application for Letters Patent No. 5864 of 1908. The steel is cast in molds having internally a formation such as to produce flat or curved armor plates of the required dimensions with, when 65 necessary, holes, recesses, projections, brackets or equivalent for engagement of the bolts or other fastening devices used for holding the plates in position on the sides of the ship. Such armor plates can readily 70 be made of different thicknesses at different parts thereof, where this is necessary, so that the metal can be disposed in the most advantageous manner to resist attack and thereby enable an effective plate to be 75 produced of the minimum weight, regard being had to the resistance which its different parts are required to offer. Thus, the armor plates, or some of them, on a battleship according to this invention can be made of 80 varying thickness in the direction of their depth, their central portions for example being of greatest thickness and their upper and lower portions of gradually diminishing thickness from the central portion. 85

My invention is shown in the accompanying drawing in which the reference characters of the description indicate corresponding parts in the different views.

Figure 1 is a face view of a plate made in 90 accordance with my invention. Fig. 2 is a vertical cross sectional view thereof. Fig. 3 illustrates in cross section a modified form of my invention and Fig. 4 shows in elevation the employment of an armor belt made 95 in accordance with my invention.

In the drawing there is shown (Fig. 2) an armor plate of the kind referred to having its central portion  $a$  of greatest thickness and its upper and lower portions  $a^1$  and  $a^2$  of 100 gradually diminishing thickness. Or, as shown in Fig. 3, each plate may be of gradually diminishing thickness at one end portion only. One or each side of such an armor plate may be made with a curved surface, as shown for example in Fig. 2, or with one or more flat surfaces as shown for example in Fig. 3. The armor plates can be made of various dimensions to suit requirement. Thus, armor plates of the kind 110 described have been produced having a depth up to between thirteen and fourteen

25 feet, a length up to twenty two feet, and of varying thickness, the weight of such a plate varying up to forty four tons in the case of a plate thirteen feet ten inches in depth, 5 twenty two feet in length; a thickness of ten inches at the central portion tapering to a thickness of four inches at the top edge and a thickness of two inches at the bottom edge. Such armor plates are or may advantageously be made of such depth, as indicated, 10 that when applied side by side to a battleship, as shown for example in Fig. 4, they will each extend the full depth of the required armor, or of the main portion of the required armor, of the ship, so that the armor, or the main portion thereof, will be composed of vertical sections only, separated by vertical division lines or joints, all 15 horizontal division lines or joints, at least in the main portion of the armor, being thereby avoided.

20 Each armor plate is or may advantageously be subjected to a special heat treatment consisting in subjecting it to successive heating and cooling operations for the purpose of increasing its toughness and resistance to perforation and fracture. For this purpose it may advantageously be subjected to the preliminary and special heat treatments to which gun house roofs are subjected as described in the said former specification. Also, the whole surface of one side of each of the armor plates, or any required part thereof, is or may be face hardened by 25 carbonizing and quenching it in an ordinary way. For example, the intermediate portion of one side of a plate made of uniform or of varying thickness as hereinbefore described, may be face hardened by 30 bedding that side of the plate which is not to be hardened, in sand on a furnace bottom, placing carbonizing material upon the intermediate portion of the other or upper surface of the plate that is to be face hardened and protecting the end portions of 35 such surface as by fire bricks or other refractory material. The side of the plate covered with the carbonizing material is then heated to a high temperature for a sufficient time to effect carbonization thereof 40 to the desired extent, and after this process is complete, the plate is quenched by water or other cooling medium either all over its surface or at that part only which has been 45 carbonized, such quenching being done either immediately after the carbonizing process is finished, or after the plate has been subjected to the special heat treatments hereinbefore mentioned. In the latter case, 50 the plate, after quenching, may be taper heated and again quenched, also in the man-

ner described in the said former specification. In this way armor plates can be produced in which the carbonizing effect will be greatest at the central portion of the 65 plate and taper off to nothing at the upper and lower ends so that they will be face hardened at the principal portion where such hardening is required and be very tough at the upper and lower ends, as well as 70 at the back of the plates. Such armor plates, whether of uniform or taper section, constitute a special feature of the invention.

By means of the present invention battleships can be built in a stronger, quicker 75 and much cheaper manner than those constructed with forged or rolled armor plates as heretofore.

Having now particularly described and ascertained the nature of the said invention 80 and in what manner the same is to be performed, I declare that what I claim is:—

1. An armor belt for battleships composed of a plurality of steel plates made of sufficient depth to extend the full depth of 85 the required armor-belt so that the said belt has vertical divisional lines only, said plates being formed of gradually diminishing thickness from their central portion.

2. A battleship having an armor belt composed of cast nickel, chromium, steel alloy plates, said plates being heat treated to produce hardened central face portions, and having toughened end portions.

3. In an armor belt for battleships, composed of a plurality of steel plates the intermediate portion of one side of each plate being carbonized and face hardened at its central portion and the carbonizing and hardening effect tapering off to nothing at 100 the upper and lower ends so that the plate will be face hardened at its central portion and be very tough at the upper and lower ends as well as at the back thereof, substantially as described.

4. A battleship provided with armor built up of plates composed of "Era steel" cast to shape and of different thicknesses in the direction of their depth, such plates being heat treated, having hardened central face 110 portions and toughened end portions and of such depth that they each extend the full depth of the required armor, or of the main portion of the required armor, of the ship, substantially as described.

115 In testimony whereof I have signed my name to this specification in the presence of two subscribing witnesses.

ROBERT ABBOTT HADFIELD.

Witnesses:

WILLIAM CROSS,  
WILLIAM CRAWLEY.